

Aug. 11, 1953

L. L. WHITNEY

2,648,750

METHOD OF MAKING A BRAKE BEAM

Filed Jan. 29, 1949



Fig. 3.

*Loren L. Whitney* INVENTOR.

BY

Wm O. S. Garner

Attij.

## UNITED STATES PATENT OFFICE

2,648,750

## METHOD OF MAKING A BRAKE BEAM

Loren L. Whitney, Hammond, Ind., assignor to  
American Steel Foundries, Chicago, Ill., a corporation of New Jersey

Application January 29, 1949, Serial No. 73,629

3 Claims. (Cl. 219—10)

1

This invention relates to the welding of truss structures, such as truss type brake beams, which are subjected in service to severe stresses, primarily compressive, along the inboard edges of the weld metal connecting the tension and compression members at the ends of the beam.

A primary object of the present invention is to devise a novel brake beam and welding method for reducing stress concentrations of the above-described type.

A more specific object of the invention is to weld the tension and compression members of the beam in such a manner as to deposit the weld metal in the form of a fillet to prevent stress concentrations therealong.

A further object of the invention is to supply molten weld metal to feed the cooling weld and prevent formation of shrinkage cracks and sinkholes therein.

The foregoing and other objects and advantages of the invention will become apparent from a consideration of the following specification and the accompanying drawings, wherein:

Figure 1 is a fragmentary plan view, partly in central horizontal section, of a welded brake beam fabricated according to the invention;

Figure 2 is a rear elevational view of the structure shown in Figure 1;

Figure 3 is an end elevational view, partly in section, on the line 3—3 of Figure 1; and

Figure 4 is a welding diagram illustrating the steps by which the novel beam is welded.

Describing the invention in detail and referring first to the brake beam structure shown in Figures 1 to 3, the beam comprises a compression member, generally designated 2, having a rear web 4 and top and bottom webs 6 and 8 respectively, the rear web being slotted as at 10 from the outboard extremity thereof. A brake head is fragmentarily indicated at 12 and comprises top and bottom ribs 14 and 16 and a portion 18 inboardly thereof sleeved or telescoped within the compression member 2 between the top and bottom webs 6 and 8 thereof. The brake head portion 18 comprises top and bottom walls 20 and 22 respectively, defining a slot 24 (Figure 3) therebetween aligned with the slot 10 of the compression member web 4. The brake head portion 18 also comprises a wall 26 connected between the top and bottom walls 20 and 22 and having a diagonal substantially flat surface 28 adapted to snugly engage a tension member 30 which, as best seen in Figures 2 and 3, is confined within the slot 24 between the top and bottom walls 20 and 22 and is also confined between the surface 55

2

28 and a parallel surface 32 of a brake head wall 34 connecting the top and bottom walls 20 and 22, as best seen in Figure 3.

The brake head 12 also comprises a portion 36 outboardly of the vertical ribs 14 and 16, the portion 36, as best seen in Figure 2, having approximately the same depth as that of the compression member and being provided with a socket 38 receiving the outboard end of the tension member 10, as best seen in Figures 1 and 2. The socket 38 comprises a diagonal surface 40 approximately coplanar with the surface 32 and, as best seen in Figure 2, comprises top and bottom surfaces 42 and 44 respectively, confining the top and bottom margins of the tension member 30.

The outboard end of the tension member is sheared as at 46 to afford a rear edge arranged diagonally with respect to the compression member wall 4 and thereby defining the inner extremity of a pocket or cavity defined by the slots 10 and 24 and the tension member 30, said pocket being adapted to contain weld metal indicated at 48 in Figure 1 fusing the tension and compression members and the brake into an integral truss structure.

As best seen in Figure 1, the weld metal at 48 is formed with a fillet 50 between the compression member web 4 and the tension member 30. This construction prevents the concentration of stresses primarily compressive in character, as the brake head 12 is applied in service to an associated railway wheel and axle assembly (not shown) in a manner well known to those skilled in the art. A primary feature of the present invention resides in the discovery that welded truss type beams, such as those heretofore known in the art, have inadequate resistance to fatigue, due to concentration of compressive stresses in the inboard edge of the weld metal connecting the compression and tension members. This difficulty has been remedied by providing a fillet in the inboard edge of the weld metal, as indicated at 50 in Figure 1. Beams of this type have disclosed remarkable resistance to fatigue such as that encountered in repeated applications of the beam in railway service to decelerate an associated wheel and axle assembly (not shown).

Referring now to Figure 4 which is a welding diagram illustrating the novel method by which the brake beam shown in Figures 1 to 3 is fabricated, it may be noted that the weld 48 may be of any conventional arc type but is preferably of the type disclosed in United States Letters Patent No. 2,043,960, issued June 9, 1936, to Union Carbide and Carbon Corporation. The welding

technique disclosed in the above-identified patent as applied to a brake beam such as that shown in Figures 1 to 3, comprises connecting the beam parts, which are steel, to one terminal and a weld electrode to another terminal of a conventional voltage supply. The electrode is positioned within the slots 10 and 24 and a readily fusible conductor, such as a piece of steel wool, may be placed between the electrode and the tension member 30 to establish an arc. However, the conductor may be eliminated by momentary use of a high frequency current to establish the arc. The slots 10 and 24 are filled with a prefused powdered welding composition of the characteristics described in the patent, the composition being electrically conductive when molten and being readily fusible at the temperature developed upon closing of the electrical circuit through the brake beam and electrode.

The novel welding process of the present invention is initiated, as will be understood by reference to Figure 4, by closing the welding circuit with the electrode extending into the slots 10 and 24 at the point indicated by the numeral 52 approximately midway between the inboard and outboard ends of the slots and the electrode is passed in the direction of the arrows from point 52 to the inboard end of the slot at a rate of speed accommodating a layer of weld metal from the point 52 to the point 54 which is at the inboard end of the slots. The electrode is then held stationary without breaking the welding circuit to establish a plug weld at 54 for a brief period of time preferably of the order of three to six seconds. The welding circuit is then broken for a brief pause of the order of three to six seconds while the electrode is moved outboard to a point indicated at 56 in Figure 4, which point is substantially outboard the inboard ends of the slots. After the pause, the welding circuit is again established with the electrode at point 56 from which the electrode is moved in the direction of the arrows to the outboard end of the slots at a rate of speed accommodating a second layer of weld metal on top of the first and fusing therewith. Then the welding circuit is again broken for a brief pause of the order of three to six seconds while the electrode dwells at the outboard ends of the slots, and after this second pause, the third pass of the electrode is initiated by establishing the welding circuit with the electrode at the outboard end of the slots, and moving the electrode in the direction of the arrows 58 to the inboard end of the slots at a rate of speed accommodating a third layer of weld metal deposited on top of the second layer.

After the electrode, at the end of its third pass, has reached the inboard ends of the slots, the welding circuit is again broken for a brief pause of the order of three to six seconds and thereafter the circuit is again closed with the electrode at the inboard end of the slots from which it is moved in the direction of the arrows 60 on the fourth or last pass at a rate of speed accommodating a fourth layer of weld metal deposited on top of the third layer. The last pass of the electrode is preferably terminated approximately midway intermediate the inboard and outboard ends of the slots, and the circuit is again broken for a pause of the order of three to six seconds whereupon the circuit is again closed for a period of about three to six seconds with the electrode stationary intermediate the ends of the slots to provide a weld puddle indicated at 62. The circuit is then broken and pref-

erably after a pause of the order of three to six seconds, the circuit is again closed for a period of about three to six seconds with the electrode stationary to provide another weld puddle intermediate the ends of the slots, as indicated at 64 (Figure 4).

It may be noted that the plug welds following the fourth pass of the electrode, which is in effect a half pass from the inboard ends of the slots to a point approximately intermediate the ends thereof, affords a pool of molten weld metal constituting a reservoir adapted to feed the cooling weld to prevent formation of shrinkage cracks therein. It may be noted that the structure shown in Figures 1 to 3 is normally welded with the slots 10 and 24 facing upwardly and the tension member surface 46 at the bottom of the slots so that the reservoir of molten metal provided by the plug welds at 62 and 64 feeds downwardly by force of gravity to the cooling weld metal.

The pause at the end of each pass permits the weld metal to partially cool, and the succeeding pass fills in any cracks which may develop in the cooling weld metal. The plug welds at the end of the last pass provide a reservoir of molten metal which as above described prevents formation of cracks in the cooling weld metal.

The above-described process results in a weld which shows no layers under microscopic examination but is a homogeneous solid weld without the slightest trace of shrinkage cavities or sink holes formed during cooling of the weld metal. Furthermore, this process provides a fillet, indicated at 50 in Figures 1 and 4, preventing concentration of compressive stresses in the inboard edge of the weld metal during application of the beam in service.

It may be noted that the engagement of the tension member with the diagonal surfaces 28, 32, and 40 and with the surfaces 42 and 44 and the complementary flat surfaces of the brake head walls 29 and 22 prevents escape of the molten weld metal during the welding operation.

I claim:

1. A method of welding a brake beam tension member within relatively telescoped brake head and compression members defining an elongated cavity with the rear surface of said tension member, said method comprising positioning an electrode in said cavity at a point between its ends, then closing an electrical welding circuit through said electrode and depositing a layer of weld metal in the cavity by passing the electrode lengthwise of the cavity to approximately the inboard end thereof, then holding the electrode stationary at said inboard end of said cavity for a period of time of the order of at least three seconds to form a puddle of weld metal at the inboard end of said cavity, then breaking said circuit and moving the electrode outboardly in said cavity to a point between the first mentioned point and the inboard end of the slot, then establishing another electrical welding circuit through the electrode and depositing another layer of weld metal on the top of the first mentioned layer by passing the electrode outboardly of said cavity lengthwise thereof to a point outboardly of the first mentioned point, then breaking the last mentioned circuit for a time interval of the order of at least three seconds, then closing another electrical welding circuit through the electrode and depositing another layer of weld metal on top of the first two layers by passing the electrode lengthwise of said cavity to a point inboardly of the second mentioned point, then

breaking the last mentioned circuit for a time interval of the order of at least three seconds without substantially moving said electrode, then closing another electrical welding circuit through said electrode and depositing a top layer of weld metal in said cavity by moving the electrode lengthwise of the cavity to a point between the inboard and outboard ends of the cavity, then breaking the last mentioned circuit for a time interval of the order of at least three seconds, and then, before the layers have solidified, establishing another electrical welding circuit through said electrode while holding the electrode substantially stationary at approximately the last mentioned point until a weld puddle has formed at said last mentioned point to feed shrinkage in the layers of weld metal.

2. A method of welding a brake beam tension member to brake head and compression members, at least one of which defines an elongated cavity with said tension member, said method comprising positioning an electrode in said cavity, then closing an electrical welding circuit through said electrode and depositing a layer of weld metal in the cavity by passing the electrode lengthwise of the cavity to approximately the inboard end thereof, then holding the electrode stationary at said inboard end of said cavity for a period of time of the order of at least three seconds to form a puddle of weld metal at the inboard end of the cavity, then breaking said circuit and moving the electrode outboardly in said cavity lengthwise thereof to a point outwardly of the inboard end of said cavity, then establishing another electrical welding circuit through the electrode and depositing another layer of weld metal on top of the first mentioned layer by passing the electrode outboardly in said cavity lengthwise thereof, then depositing another layer of weld metal on top of the first two layers by passing the electrode lengthwise of said cavity to a point inboardly of said first mentioned point until a weld puddle has formed to feed shrinkage in the layers of weld metal.

3. A method of welding a brake beam tension member to brake head and compression members, at least one of which defines an elongated cavity with an edge of said tension member, said

method comprising positioning an electrode in said cavity, then closing an electrical welding circuit through said electrode and depositing a layer of weld metal in the cavity on top of said edge by passing the electrode lengthwise of the cavity to approximately the inboard end thereof, then holding the electrode approximately stationary at said inboard end of said cavity for a period of time of the order of at least three seconds to form a puddle of weld metal at said inboard end of said cavity, then breaking said circuit and moving the electrode outboardly in said cavity lengthwise thereof to a point outboardly of the inboard end of said cavity, then establishing another electrical welding circuit through the electrode and depositing another layer of weld metal on top of the first mentioned layer by passing the electrode outwardly in said cavity lengthwise thereof, and then depositing another layer of weld metal on top of the first two layers by passing the electrode inboardly lengthwise of said cavity to a point inboardly of said first mentioned point.

LOREN L. WHITNEY.

25 References Cited in the file of this patent

UNITED STATES PATENTS

| Number    | Name           | Date           |
|-----------|----------------|----------------|
| 461,776   | Alley -----    | Oct. 20, 1891  |
| 1,290,091 | Cole -----     | Jan. 7, 1919   |
| 1,290,093 | Cole -----     | Jan. 7, 1919   |
| 1,293,871 | Murry -----    | Feb. 11, 1919  |
| 1,634,995 | Huntoon -----  | July 5, 1927   |
| 1,810,905 | Burnish -----  | June 16, 1931  |
| 1,939,732 | Stresau -----  | Dec. 19, 1933  |
| 2,141,021 | Rooke -----    | Dec. 20, 1938  |
| 2,177,927 | Hodge -----    | Oct. 31, 1939  |
| 2,239,186 | Anderson ----- | Apr. 22, 1941  |
| 2,262,212 | Stone -----    | Nov. 11, 1941  |
| 2,356,720 | Aurien -----   | Aug. 22, 1944  |
| 2,371,823 | Jackson -----  | Mar. 20, 1945  |
| 2,416,379 | Cohn -----     | Feb. 25, 1947  |
| 2,473,002 | Baselt -----   | June 14, 1949  |
| 2,500,232 | Baselt -----   | Mar. 4, 1950   |
| 2,517,747 | Whitney -----  | Sept. 18, 1950 |

FOREIGN PATENTS

| Number  | Country      | Date          |
|---------|--------------|---------------|
| 618,890 | France ----- | Dec. 21, 1926 |

50 OTHER REFERENCES

The Welding Engineer, Aug. 1944, page 37.  
Procedure Handbook of Arc Welding Design and Practice, 8th ed., 1945, pages 34 and 166.